

## UNITED STATES PATENT OFFICE

2,488,618

LUBRICANTS OF THE EXTREME PRESSURE  
TYPE

Elmer B. Cyphers, Cranford, and George M. McNulty, Union, N. J., assignors to Standard Oil Development Company, a corporation of Delaware

No Drawing. Application November 25, 1946,  
Serial No. 712,050

4 Claims. (CL. 252—46.6)

1

The present invention relates to lubricants of the extreme pressure type and particularly to extreme pressure lubricants containing materials such as phosphorus, sulfur and compounds thereof in mineral and/or fatty oil bases.

In many types of modern machinery very high unit pressures occur between the adjoining surfaces of moving metallic parts. Unless such surfaces are effectively and continuously lubricated, rapid wear and early destruction occur. At the pressures which are sometimes employed, and particularly when metal parts such as hypoid gears in automotive vehicles are operated at high speeds, or, more particularly, at high torques, as in heavy duty automotive vehicles, conditions arise where ordinary lubricants are not capable of maintaining effective lubricating films. Momentary rises in temperature also cause the protective oil film to separate and, in extreme pressure lubricants, materials are provided which, on such momentary rise of temperature, will react with the metal to form thin protective layers of chemical reaction products. Thus, as is well known in the art, certain substance such as sulfur, chlorine, phosphorus and the like, when added to lubricating oils and when rendered reactive by rise in temperature, combine in some chemical manner with the metal to produce protective films of approximately molecular thickness or thickness of that general order. These films adhere tenaciously to the metal, preventing metal to metal contact momentarily until the normal oil film can be restored.

Lubricants of the general character referred to above usually consist of blends of petroleum oil with a saponifiable oil, usually an animal or vegetable oil, containing as extreme pressure agents either free elements or chemical compounds of sulfur, chlorine, phosphorus and related materials. It is desirable that at ordinary temperatures these materials be relatively inactive, being adapted to react vigorously with the metal surfaces upon temperature increases which result, as on momentary failure of the lubricating oil film.

In the past, it has been necessary to compromise between extreme pressure additives which, on the one hand, are effective when needed to provide the type of chemical film mentioned above, but are objectionably corrosive, over a period of time, to metals such as copper and steel, and those, on the other hand, which are relatively non-corrosive but are only moderately effective as extreme pressure agents.

The thin protective films referred to above

probably consist of metal sulfides, chlorides, phosphides and the like. Thus when materials such as sulfur, chlorine or phosphorus are used in an active form in a lubricant for steel gearing, iron sulfides, chlorides or phosphides may be formed on the gear teeth. Analogous reactions occur with other metals and with other extreme pressure additives.

In the past, numerous compounds have been used for the purpose described above; among them are not only inorganic materials such as free sulfur, free phosphorus, sulfides, etc., but also aryl and alkyl chlorides and various other organic as well as inorganic compositions of sulfur, phosphorus, chlorine, arsenic, selenium, lead, etc. These materials have usually been added to fatty oils which in themselves have certain extreme pressure properties. Certain animal and vegetable oils have very desirable film strength properties but often are somewhat unstable and in some respects not entirely satisfactory as lubricant additives. It is therefore an object of the present invention to use materials other than, or in addition to, fatty oils in mineral oil lubricating compositions, as extreme pressure additives.

A further object is to combine certain organic materials which have been found desirable substitutes for fatty materials, with sulfur- or phosphorus-containing materials in a manner to provide extreme pressure lubricants and additives therefor having useful and superior properties.

Still a further object is to use organic materials in lubricants which have certain economic advantages over fatty oils and the like previously used in lubricants of the general character to which this invention pertains. The materials proposed for use according to the present invention are, in some instances, at least less costly and in some cases more abundant than fatty materials conventionally used.

We have discovered that by treating certain esters of abietic acid, or hydrogenated abietic acid with phosphorus-containing materials, lubricants may be produced which have useful extreme pressure properties and which are free from certain of the objections to which fatty oils are subject. Also, in lieu of simple esters of abietic acid or hydrogenated abietic acid, sulfurized esters of the same may be combined with phosphorus containing materials.

In a copending application, Serial No. 708,794, filed November 8, 1946, by Elmer B. Cyphers and Louis J. Osborne, there is disclosed an extreme

pressure lubricant and a process for producing the same which involves the use of sulfurized and phosphorized fatty oils to which an organic phosphorus compound is added. As described in said application, the fatty oils may be treated with free sulfur and a phosphorus sulfide, such as  $P_4S_3$ , may be added thereto, the phosphorus sulfide being particularly useful as an extreme pressure ingredient. As a suitable organic phosphorus compound, tricresyl phosphate has been found useful since it has desirable properties as an "oiliness" agent and also as an anti-oxidant. In lieu of tricresyl phosphate, various esters of phosphoric and phosphorous acids may be used as organic additives, and the substitution of hydrogen atoms in such materials by alkyl or aryl additives, to form either complete or partial esters, is contemplated.

The process just described is also applicable to esters of abietic acid, hydrogenated abietic acid or sulfurized esters of the same. It is to be understood, however, that the present invention is not dependent upon the use of a second added phosphorus compound such as tricresyl phosphate and the like, although such may be used if desired to improve the effectiveness of our compositions. A suitable composition may be provided by merely treating the esters or sulfurized esters of abietic acid and/or hydrogenated abietic acid with phosphorus-containing materials such as the phosphorus sulfides as, for example,  $P_4S_3$ . Other phosphorus compounds, such as  $PCl_3$ ,  $PCl_5$ ,  $POCl$ ,  $POCl_3$ ,  $PO_2Cl$ ,  $P_2O_5$ ,  $P_2O_3$ , etc. may be employed but we prefer to use the phosphorus sulfide such as  $P_2S_5$ ,  $P_4S_7$  and  $P_4S_3$ , the last being particularly preferred.

The abietic acid derivatives mentioned above have a notable advantage over the fatty oils conventionally used in extreme pressure lubricants as regards treatment with phosphorus sulfides. Fatty oils must be sulfurized, for example, by cooking free sulfur into them, before they can be treated satisfactorily with a phosphorus sulfide such as  $P_4S_3$ . The abietic acid derivatives, however, can be treated directly and the reaction product is found to be a rather effective extreme pressure agent, capable of carrying fairly high loads.

It will be understood that an extreme pressure additive such as described above, consisting of alkyl esters of abietic acid, and related compounds reacted with phosphorus-containing materials, is not only useful in lubricants designed especially for extreme pressure functions, but may be useful generally in various types of lubricating oils and greases. Thus it may be used in mineral oils, fatty oils, or synthetic oils, or mixtures thereof. It may be used in greases prepared, for example, by the addition of soaps to lubricating oils, or by the addition of carbon black and like thickeners to oils. It may be used alone or in conjunction with other extreme pressure additives and along with corrosion inhibitors, anti-oxidants, pour point depressants and the like, as will be readily understood in the art.

Ordinarily the material resulting from the reaction of methyl abietate and the like with a phosphorus sulfide will be used in quantities of 5 to 15%, based on the total lubricant, but these proportions may be varied widely. As little as 0.5% or as much as 20% or more may be required under some conditions. When incorporated in a grease embodying material quantities of soaps or other thickeners, the base lubricating oil content may be as little as 60%. In oils, the

base lubricant will usually run 80% or more, to as much as 99.9%. Specific examples of suitable compositions are as follows:

#### EXAMPLE 1

940 grams of a commercial grade of methylated rosin produced by esterification of rosin with methyl alcohol was heated in an open beaker to 280° F. and 60 grams of sulfur added with good agitation. Such a material is sold commercially by the Hercules Powder Company under the trade name "Abalyn." The temperature was raised to 385° F. and held at this point for 2 hours, after which the sulfurized product was cooled. Next day it was heated at 210° F., 5 grams of phosphorus sesquisulfide was added, and the temperature was maintained at 210-220° F. for eight hours with continuous agitation, followed by natural cooling.

10 parts of the above product were blended with 90 parts of SAE 90 grade mineral oil and the blend was tested on the Timken machine with the results shown in the table.

#### EXAMPLE 2

1940 grams of the same commercial rosin derivative methyl abietate and 60 grams of sulfur were charged to an autoclave. The autoclave was then flushed with nitrogen and the outlet closed and nitrogen charged to 10 lbs. gauge pressure. Heat and stirring were applied to raise the temperature to 330° F. in one hour and a temperature of 320-330° F. and gauge pressure of 10 lbs. maintained for 5 hours. The sulfurized product was then removed and cooled, after which 4 grams of phosphorus sesquisulfide were added to 1000 grams of the sulfurized product, and the mixture stirred and heated in an open beaker at 210-220° F. for five hours.

10 parts of the resulting product and 90 parts of the SAE 90 grade mineral oil were blended and tested on the Timken machine with the results shown in the table below.

#### EXAMPLE 3

6 grams of phosphorus sesquisulfide and 294 grams of a methyl dihydroabietate, produced by the methylation of rosin, were mixed and heated in an open beaker to 300° F. in one hour and then held at 300° F. for 1/2 hour. Such a hydrogenated and methylated rosin as just described is available commercially being sold under the trade name "Hercolyn" by the Hercules Powder Company. 10 parts of the resulting product and 90 parts of the SAE 90 grade mineral oil were blended and tested with the results shown in the table.

TABLE

Timken machine test data

|     | Lubricant                                                      | OK Load, Lbs. | Scar Width, in 64th Inch | Unit Load, Lbs./sq. in. |
|-----|----------------------------------------------------------------|---------------|--------------------------|-------------------------|
| 60. | SAE 90 Grade base oil.....                                     | 10            | 1.65                     | 7,800                   |
| 65. | 10% Example 1 in above base oil.....                           | 43            | 1.65                     | 33,400                  |
|     | 10% Example 1+0.1% tri-cresyl phosphate in above base oil..... | 51            | 1.65                     | 39,500                  |
| 70. | 10% Example 2 in above base oil.....                           | 43            | 2.2                      | 25,000                  |
|     | 10% Example 2+1.0% tri-cresyl phosphate in above base oil..... | 51            | 1.8                      | 36,300                  |
| 75. | 10% Example 3 in above base oil.....                           | 43            | 2.4                      | 22,900                  |
|     | 10% Example 3+0.1% tri-cresyl phosphate in above base oil..... | 51            | 2.1                      | 31,100                  |

The SAE 90 grade oil referred to in the above example consisted of 49.75% of a conventional Mid-Continent steam cylinder oil and 49.75% of an SAE 20 grade solvent extracted Mid-Continent oil, together with 0.5% of a conventional pour point depressant. The methylated rosin or methyl abietate, mentioned in Example 1 is a proprietary product of the Hercules Powder Company. It is understood to be produced by the esterification of rosin, which is largely abietic acid, with methyl alcohol. Its composition is believed to be substantially as follows:

|                                                                                             | Per cent |
|---------------------------------------------------------------------------------------------|----------|
| Methyl esters of abietic and neoabietic acid<br>(contain 2 conjugated double bonds per mol) | 23       |
| Methyl ester of dihydroabietic acid (contains 1 double bond per mol)                        | 22       |
| Methyl ester of tetrahydroabietic acid (contains no double bonds)                           | 22       |
| Methyl ester of dehydroabietic acid (contains one benzenoid ring)                           | 17       |
| Unsaponifiable matter (pinenes, ethers, etc.)                                               | 16       |
|                                                                                             | 100      |

This composition may be described roughly as a methyl abietate or more accurately as a methyl ester of rosin having an average double bond content of approximately 0.80 active double bond per mol not counting benzene type bonds. The ester of Example 1 has an average value of 8.0 and an equivalent molecular weight of 358 based on the saponification value determination.

In lieu of the methyl abietate the related material mentioned above in connection with Example 3 may be used. This is also a proprietary product marketed by the Hercules Powder Company. Whereas the former appears to be a mixture of methyl esters of abietic acid derivation, the latter is somewhat more fully hydrogenated, having roughly the following formula:



It will be noted that hydrogenated and methylated rosin is more fully saturated than methylated rosin. These materials appear to have certain desirable surface tension properties which make them useful as lubricating film forming or film strengthening agents. By reason of the limited extent of their unsaturation, they are quite stable and because of their film strength properties, they appear to combine effectively in lubricants to produce desirable extreme pressure compounds, especially when combined with additives of the phosphorus sulfide type. As indicated above, they appear to be superior to fatty oils in that they can be treated directly with a phosphorus sulfide without sulfurization.

It will be understood from the foregoing that the esters and sulfurized esters of abietic acid have been found to serve very satisfactorily as substitutes for fatty oils and sulfurized fatty oils which in the past have been considered essential in certain types of lubricants. By the use of these materials, unstable fatty bodies may be eliminated from oils and greases while their desirable oiliness and film forming characteristics may be retained. It will be understood, however, that the

abietic acid esters, sulfurized or otherwise, are compatible with fatty bodies and may be used in conjunction with vegetable and/or animal oils as well as in mineral oils with or without fatty constituents.

Thus, a satisfactory lubricant may be formed by combining sulfurized or unsulfurized the methylated rosin, referred to generally herein as a methyl abietate, or methylated hydrogenated abietate, referred to herein by its approximate formula methyl dihydro abietate, with phosphorus sesquisulfide, or other phosphorus sulfides, with or without the addition of tricresyl phosphate or an analogous phosphorus containing organic compounds.

Various other organic abietates, such as other alkyl esters of abietic acid may be used. It will, of course, be understood that materials as described above may be included in oils containing or even consisting largely or entirely of fatty oils, sulfurized fatty oils and the like. Sulfurized mineral oils, which themselves have mild extreme pressure properties, may also be so treated, and the percentage of sulfur in active form may be up to or exceeding 1%.

Extreme pressure compositions consisting of mineral and/or fatty oils including various percentages of the materials described above may be used per se as lubricants or may be added to lubricating oils in various proportions to secure the characteristics desired for a particular purpose. Synthetic oils of the ethylene glycol type, for example, may be used in lieu of or in addition to mineral and/or fatty oils. Referring to the example given above when 10% of P4S3 treated sulfurized commercial methyl abietate so-called was added to SAE 90 grade base oil, it will be noted that the load carrying characteristics were considerably increased by the addition of 0.1% of tricresyl phosphate. For some purposes, the use of the latter material may not be necessary or desirable but it appears to have merit where high load carrying qualities are required and where corrosivity must be held to a minimum. Since it is usually desirable to keep corrosivity to a minimum while imparting extreme pressure qualities to a lubricant, it will frequently be found advantageous to add a part of the reactive phosphorus in the form of an organic phosphate or phosphite, as described in the above mentioned copending application of Cyphers and Osborne.

The quantity of organic phosphate or phosphite which may be included in compositions according to the present invention may vary considerably. Ordinarily a small amount is sufficient, suitable percentages being from 0.01 to 5%, based on the total composition.

The amount of the phosphorus sulfide treated abietic ester may vary from as little as 0.5 to 20% or more, based on the total composition. The reaction product may be sulfurized after the reaction has been completed, in the same manner that fatty oils are commonly sulfurized. Such a sulfurized product may be found to have desirable extreme pressure properties for certain applications.

As indicated above, this invention deals broadly with the addition of the reaction products of phosphorus sulfides with esters of abietic acid to lubricants of various types. Mineral oils, synthetic oils, fatty oils, and greases comprising various bodying agents may be treated with various quantities of such reaction products, depending on their respective characters and purposes. The reaction between the phosphorus sulfides and

the various abietic acid derivatives enumerated hereinabove appears to proceed over a rather wide temperature range and the invention is not to be limited either to the specific compositions or the reaction conditions mentioned hereinabove. Thus reactions may proceed at moderate temperatures, 60° F., for example, or at any temperatures up to 400° F. or more. The derivative of abietic acid, whether of the methyl ester type or the dihydro-methyl ester type, as described above, or related composition, may be sulfurized by heating with sulfur as is common practice with fatty oils and mineral oils, and this may be effected either before, during or after treatment with a phosphorus sulfide. The time of heating will be varied as required to obtain a reaction product which is effective as an extreme pressure agent.

The methylated and hydrogenated abietic acid derivatives mentioned above appear to be excellent for the purposes of the present invention, but ethyl and higher alkyl esters of abietic acid, sulfurized abietic acid, hydrogenated abietic acid and its esters, and the like are contemplated as being within the spirit of our invention.

While we have described our invention in terms of specific compounds prepared in specific ways, the invention is not limited thereto or otherwise, except as indicated in the appended claims.

We claim:

1. A composition consisting essentially of 80 to 99.5% of petroleum base lubricating oil and 0.5 to 20% of the phosphorus-containing reaction product of a sulfide of phosphorus with a methyl ester of abietic acid which has been substantially

5 saturated with a material selected from the class which consists of hydrogen and sulfur, said reactant ester and sulfide of phosphorus being reacted for a substantial period of time at a temperature between about 60° F. and about 300° F.

2. An extreme pressure lubricating composition consisting essentially of 80 to 99.5% of petroleum base lubricating oil and 0.5 to 20% of the phosphorus-containing reaction product of P<sub>4</sub>S<sub>3</sub> with a material selected from the class which consists of hydrogenated methyl esters of abietic acid and sulfurized methyl esters of abietic acid, said reactants being reacted for a substantial period of time at a temperature between about 60° F. and about 300° F.

3. A composition as in claim 1, wherein the material reacted with phosphorus sulfide is sulfurized "Abalyn."

4. A composition as in claim 1, wherein the material reacted with phosphorus sulfide is "Hercolyn."

ELMER B. CYPHERS.  
GEORGE M. McNULTY.

#### REFERENCES CITED

The following references are of record in the file of this patent:

#### UNITED STATES PATENTS

| Number    | Name                   | Date          |
|-----------|------------------------|---------------|
| 2,252,133 | Morway et al. -----    | Aug. 12, 1941 |
| 2,347,592 | Cook et al. -----      | Apr. 25, 1944 |
| 2,357,211 | Lincoln et al. -----   | Aug. 29, 1944 |
| 2,415,837 | Musselman et al. ----- | Feb. 18, 1947 |